

## UNITED STATES PATENT OFFICE

JOHN PARSONS, OF NEWTON CENTER, MASSACHUSETTS, AND JORDAN HOMER STOVER, OF NUTLEY, NEW JERSEY, ASSIGNEES, BY DIRECT AND MESNE ASSIGNMENTS, TO PAN-ROSS LABORATORIES, INC., OF NEW YORK, N. Y., A CORPORATION OF NEW YORK

## IGNITING COMPOSITION

No Drawing.

Application filed September 5, 1925. Serial No. 54,796.

This invention relates to new and useful improvements in igniting compositions, and has for its object the providing of an igniting composition particularly adapted for use in connection with fuse bands capable of use in the making of self-lighting cigarettes, cigars and little cigars. It is also capable of many other uses.

The invention consists in the novel compositions hereinafter described and claimed, but it is not intended that the invention be limited to the particular preferred form set forth, but the scope of the invention is as set forth in the claims.

15 We have found that if, in the manufacture of igniting compositions, a substance such as nitrocellulose is used, a composition is formed peculiarly adapted for use in connection with self-lighting cigarettes and with fuse bands 20 adapted to be attached to the ends of such cigarettes. A preferred form of making an ordinary strike-anywhere igniting composition embodying our invention is as follows: Four parts of potassium chlorate or other 25 suitable oxidizer in proper proportion, one part of sulphur, three parts of a frictionizer such as ground glass, and one-half part of a substance such as red phosphorus are thoroughly mixed together in dry form. Two 30 parts of the powder are then mixed with one part of nitrocellulose dispersion or solution of a consistency of 12 ounces of nitrocellulose to a gallon of the solution in a dispersing agent such as benzol and ethyl acetate. The 35 resulting mixture may be then spread on a previously-prepared fuse band, and, as the dispersing agent evaporates, the powdered igniting composition will be finely spread over such surface, being bound by the nitrocellulose, and will serve as an igniting composition for same when rubbed against any 40 abrasive surface.

This form of igniting composition is particularly adapted for use with a fuse composition described in an application filed on even date herewith.

In lieu of spreading the igniting composition on top of a previously-prepared fuse composition, the fuse composition and the igniting composition may be mixed together

and a single spread made of both the fuse composition and the igniting composition.

Whether the igniting composition be spread on the fuse composition or be mixed with same, an advantageous combination will result, inasmuch as both the fuse composition and the igniting composition are held by a similar form of binding agent which will render the binding agent of the entire mass homogeneous.

Furthermore, the use of a plastic self-oxidizing binder for an igniting composition renders the same more effective, inasmuch as the binder itself is highly combustible and is provided with its own oxidizing influences, and also the igniting composition is rendered largely impervious to moisture by the moistureproofing qualities of the nitrocellulose. Other plastic binding substances may be substituted for the nitrocellulose with somewhat similar results, as same are combustible and self-oxidizing or are provided with an oxidizing agent.

A safety form of igniting composition may be made in accordance with our invention by mixing together potassium chlorate eighteen parts, manganese dioxide and iron peroxide two parts each, bichromate of potash one and seven-tenths parts, sulphur powder one part, and ground glass four parts. After same have been thoroughly mixed in dry form, the powder is mixed in ten parts with seven parts of nitrocellulose solution of a consistency of that previously described, and five additional parts of a dispersing agent as ethyl acetate are added thereto. These ingredients are thoroughly mixed in a receptacle, allowed to stand and drawn from the bottom and spread over a fuse band forming a thin lamination thereon, or may be mixed in with the fuse composition before spreading, or may be used in other ways. Here again the usual comminuted ingredients of safety igniting compositions have been mixed and held by a plastic binder which is self-combustible or mixed with an oxidizing influence, and the preferred form of such a substance is the nitrocellulose solution described, although other materials may be substituted as in the case of the strike-anywhere igniting composition.

The igniting composition will ignite on any common safety match striking abrasive. A striking surface for the igniting composition, however, may be composed of a frictionizer of twelve parts of glass powder mixed with five parts of red phosphorus, and cemented with four parts of nitrocellulose solution of a consistency previously described. The mixture is thinned with ethyl acetate for suitable spreading, and may, if desired, be darkened with lamp black, red oxide or other coloring matter. The use of a substance such as nitrocellulose in the abrasive surface renders same moisture proof and, being itself combustible and self-oxidizing, likewise aids in the ignition of the igniting composition by more freely liberating the spark on striking. Instead of retarding ignition as do the ordinary glues used as binders, the nitrocellulose binder itself generates heat at the friction point. This enables the igniting composition to be ignited with less friction.

The nitrocellulose as used in the igniting compositions and in the striking surface described not only serves as a binder for the ingredients in such substances, but, being itself a transporter of combustion and self-combustible, it effectively aids in the proper action of the igniting compositions. It is also plastic and renders the mixtures flexible and capable of being manipulated into ribbon form. It also renders the mixtures moisture-proof.

What we claim as new and desire to secure by United States Letters Patent is:

1. A safety igniting composition for self-lighting cigarettes, cigars and the like consisting of potassium chlorate, manganese dioxide, iron peroxide, potassium bichromate and sulphur, agglutinated with a nitro-cellulose substance into a plastic compound.

2. A safety igniting composition for self-lighting cigarettes, cigars or the like consisting of ten parts of powder formed from eighteen parts of potassium chlorate, two parts of manganese dioxide and iron oxide each, one and seven-tenths parts of potassium bichromate, one part of sulphur and four parts of ground glass; and seven parts of nitro-cellulose dispersion of consistency of substantially twelve ounces of nitro-cellulose to a gallon of dispersing agent.

In testimony whereof, we have signed our names to this specification.

JOHN PARSONS.

JORDAN HOMER STOVER.